

B. TALBOT.

STEEL SHAPE.

APPLICATION FILED NOV. 6, 1912.

1,055,832.

Patented Mar. 11, 1913.

*Fig. 1.*



*Fig. 2.*



*Fig. 3.*



*Fig. 6.*



*Fig. 4.*

WITNESSES:

*Joe G. Denney*  
*Bro. Denney*

INVENTOR

*Benj. Talbot*  
BY  
*Charles N. Butler*

ATTORNEY.

# UNITED STATES PATENT OFFICE.

BENJAMIN TALBOT, OF WOODBURN, DARLINGTON, ENGLAND.

## STEEL SHAPE.

1,055,832.

Specification of Letters Patent. Patented Mar. 11, 1913.

Application filed November 6, 1912. Serial No. 729,765.

*To all whom it may concern:*

Be it known that I, BENJAMIN TALBOT, a British subject, residing at Woodburn, Darlington, Durham county, England, have 5 invented new and useful Improvements in Steel Shapes, of which the following is a specification.

My invention relates more particularly to railway rails and has as its primary object 10 to improve the structure of the metal of the usual steel rail so that it shall be free from flaws and defects and possessed of a uniformly tough interior lower in carbon than the outer strata. 15 Steel rails frequently contain hidden flaws and structural defects due to blow holes, cavities and segregates, which have resulted in many serious accidents. Usually the carbon in the central part of the upper third of 20 the ingot is higher than in the outer strata, which produces a rail or rails having harder interior sections than the exteriors subject to wear, which is the reverse of the desired conditions. These defects are due to conditions 25 arising in the process of manufacture in which the ingot is formed by pouring the molten steel into a mold and allowing it to solidify without provision compensating for internal shrinkage, liberation of gas after 30 the outer strata have hardened, and segregation within the upper part of the mass. If usual cold ingots be divided longitudinally, they will be found to contain blow holes or cavities, particularly in the upper third part, 35 either scattered through the mass, or where a powerful deoxidizer has been added to the molten steel, the smaller blow holes are eliminated in great measure and large cavities or pipes are formed in the center of the upper 40 third of the ingot. In the process of cooling, carbon, sulfur and phosphorus segregate and move, as the metal cools, from the outer to the inner parts of the ingots, collecting in excess in the central part of 45 the upper third as a segregate, frequently in seriously objectionable degree. When such ingots are heated to the requisite temperature and rolled, the blow holes and cavities or pipes are found in the finished products 50 as cracks or flaws, since the metal surrounding them cannot be heated to a fluid condition, and the sections in which the excessive segregation has taken place produce sections in the finished products which are defective,

more or less of the metal in such sections 55 being brittle and treacherous.

I have found that if an ingot be stripped as soon as practicable after casting, placed in a heating furnace or soaking pit until the solidified envelop has increased in thickness 60 and become sufficiently ductile or plastic to work without cracking or rupturing, and then squeezed while its interior is still in a fluid condition so as to contract its cross-sectional area to compensate for shrinkage 65 and eliminate cavities due to confined gas and unequal cooling, it will be found that the interior of the ingot is (due to the condensing lateral pressure) solid in texture and free from blow holes, cavities or pipes 70 except in a limited end portion; that the mass of the central portion of the ingot is lower in carbon than the outer strata; that there is a slight but unobjectionable indication of segregation approximately parallel 75 to and at a short distance from the surface of the ingot; and that there is no segregation within the central mass of the ingot and no objectionable segregation elsewhere. At the end of the treatment in the soaking 80 pit, the pipe in the upper part of the ingot is partially formed and the metal between the solidified but ductile outer strata and fluid central mass has little coherence so that when the ingot in this condition is subjected to lateral pressure, as by passing it 85 through a cogging mill, the liquid metal fills the pipe and the contained gases are forced outwardly, passing through or being absorbed by the enveloping metal, while carbon, phosphorus and sulfur diffused through the congealing metal are retained, tests showing these elements in higher degree and distributed in a comparatively uniform manner through the envelop with a slightly 90 increased amount at a short distance from the surface where a segregate, if substantial in character, would be least objectionable. An ingot of this character, when rolled or drawn, will produce rails, beams and other 95 shapes or products having comparatively pure and tough interiors combined with comparatively hard exteriors, without the usual defects and with substantial economy of material since there is required to be removed but a small crop or discard, as practically the whole ingot is solid.

In carrying out my invention, I prefer to

treat the molten steel, either before or after it is poured into the ingot mold, with metallic aluminum, or other deoxidizer, such as silicon, ferro-silicon, silico-manganese or ferro-titanium, for the purpose of effecting initially the elimination of small blow holes disseminated throughout the body of the upper third portion of the ingot, and to hasten the stiffening of the metal.

10 As the objectionable cavities and segregation take place in the upper third of the ingot, I may confine the squeezing operation for the purpose of eliminating the cavities and disseminating the segregates to such 15 upper third or only the upper part of the ingot.

In steel which has been treated by an electrical refining process, the amount of segregation observed is usually very small, but 20 the cavities form in the same way as in steel made by the Bessemer or Siemens processes, and it is my purpose to produce ingots and the products thereof without the defects resulting from such cavities.

25 While it is not essential to do so in all cases, the ingots will generally, after having been subjected to the squeezing operation, be returned to the heating furnace or soaking pit, to effect a more nearly equal and desirable temperature and condition throughout 30 the mass of the metal prior to rolling or finally forming the desired shape.

In the accompanying drawings, Figure 1 is a longitudinal sectional view of a steel 35 ingot after stripping when it has a comparatively thin envelop of solid metal surrounding a fluid body; Fig. 2 is a longitudinal sectional view of the same after it has been heated in a soaking 40 pit for such time and at such temperature that the envelop has become sufficiently thick and sufficiently soft to work without rupturing; Fig. 3 is a longitudinal sectional view representing an ingot 45 or bloom that has resulted from squeezing the ingot shown in Fig. 2 by the application of lateral pressure thereto so as to reduce its cross-sectional area; Fig. 4 is a transverse 50 sectional view of a rail produced by rolling the ingot or bloom shown in Fig. 3; Fig. 5 is a transverse sectional view of an I-beam 55 rolled from an ingot or bloom like that shown in Fig. 3; and Fig. 6 is a longitudinal sectional view representing an ingot having the cross section of only its upper 60 part reduced to eliminate cavities and force the segregates outwardly.

The ingot A, shown in Fig. 1, is say 20" wide at the bottom and has an envelop a 60 which may be 1" thick, such envelop being too thin and hard for satisfactory contraction by rolling or squeezing to reduce the cross section of the ingot while its central part a' is still fluid.

65 The ingot B, shown in Fig. 2, results from

heating the ingot A until there is produced the comparatively soft or ductile and thick envelop b containing the fluid central mass b' at the top of which the cavity b<sup>2</sup> will have formed, the envelop being, say, 3" thick.

The ingot or bloom C, shown in Fig. 3, is the product resulting from giving the ingot B several passes in a cogging mill or otherwise squeezing it so as to reduce its cross sectional area, eliminate the cavities or confine them to a restricted part of the top, and provide the comparatively pure central part c surrounded by the strata c' of somewhat higher carbon, together with phosphorus and sulfur (if any), there being 70 generally a noticeable but unobjectionable stratum of segregation along the inner part c<sup>2</sup> of the strata c'. That is to say, as shown by averaging sections of a typical ingot, where the central part c contained an average of .50% carbon, .02% phosphorus and .03% sulfur, an outer stratum c' near the edge of the ingot contained an average of .70% carbon, .03% phosphorus and .04% sulfur, and a stratum c<sup>2</sup> between the foregoing parts an average of .80% carbon, .04% phosphorus and .06% sulfur.

80 It will be understood that there is no distinct or abrupt line of demarcation between the strata, which term is used here with reference to zones containing different amounts of the elements, the change in the amounts of the elements through the several strata being gradual.

The rail D, shown in Fig. 4, is the product produced by rolling the ingot or bloom C, the rail having the comparatively pure and softer central part d and the harder exterior d' providing a tough center combined with a hard wearing surface. The I-beam 100 E, shown in Fig. 5, is likewise provided with the comparatively pure and softer central or body part e with a slightly harder surface e'.

The ingot F, shown in Fig. 6, has its upper part only reduced in cross section, with resulting elimination of cavities and diffusion of the matter which would otherwise form a segregate in the center of such upper part. The lower part of the ingot will 110 be found to be in the usual condition, the center f of the upper part will be found comparatively pure, and the outer strata f' will be found to have the segregates diffused therethrough, particularly through 115 the parts thereof adjacent to the central part f.

120 It will be understood that while I have given specific illustrations of dimensions and conditions, in order to explain my invention by example, such illustrations are merely by way of example and not limiting features of my invention.

Having described my invention, I claim:

1. A steel shape having a purified central 130

part lower in carbon and phosphorus than outer strata thereof.

2. A steel shape having the segregate removed from the central part and distributed substantially parallel to a surface or surfaces thereof.

3. A steel rail having a head with a purified central part lower in carbon than the outer strata, and the segregate distributed between said central part and outer surfaces thereof.

4. A steel rail having a purified central part, an enveloping part, and a stratum of maximum carbon between the central part and the enveloping part.

5. A steel rail having a purified central part, an enveloping part higher in carbon

than said central part, and strata between said central and enveloping parts in which impurities removed from said central part are deposited.

6. A steel rail having a purified central part, an outer stratum higher in carbon than said central part, and a stratum between said central part and said outer stratum higher in carbon than said outer stratum.

In witness whereof I have hereunto set my name this 4th day of November, 1912, in the presence of the subscribing witnesses.

BENJAMIN TALBOT.

Witnesses:

Jos. G. DENNY, Jr.,  
GEO. A. CUNNEY.